

## 1

3,088,911

## LUBRICANT CONTAINING ASHLESS ANTIWEAR ADDITIVES

Gerald D. Staffin, Westfield, and Walter K. Range, Jr., Elizabeth, N.J., assignors to Esso Research and Engineering Company, a corporation of Delaware  
No Drawing. Filed Nov. 9, 1961, Ser. No. 151,168  
5 Claims. (Cl. 252—33.6)

This invention relates to improved lubricating oil compositions containing additives that function as wear-reducing agents. The antiwear additives of the invention are particularly characterized by the fact that they are metal-free, thus permitting them to be used where either ashless compositions or compositions relatively low in ash-forming tendencies are desired. The additives of this invention also have the desirable property of not contributing materially to oxidation or corrosion instability.

In the formulation of crankcase lubricants for piston-type internal combustion engines for automotive use, the recent trend has been to employ viscosity index improvers, oxidation inhibitors, and detergents in order that the lubricant may serve its purpose under a wide variety of conditions, including high-speed driving for sustained periods as well as low-speed stop-and-go driving at relatively low temperatures. The detergents and oxidation inhibitor additives enable the oil to keep the various parts of the engine free of varnish and cokelike deposits. At the same time, these additives prevent or at least minimize the formation of sludge and also hold in suspension any sludge that may be formed. There is one major disadvantage to detergents and inhibitors in crankcase lubricants, however, and that is that they keep the wearing surfaces of the engine particularly clean. For this reason, they contribute to a higher degree of wear than would occur if there were no detergents and inhibitors present. This problem of wear with high detergency oils shows up particularly in the valve train of automotive engines and especially in the valve lifter mechanism. In the valve lifter mechanism, pressures as high as 100,000 lbs. per square inch can exist between the valve lifter and its actuating cam. For this reason, in present-day high detergency crankcase lubricants, there is a need for antiwear additives.

While in the past certain metal salts such as molybdenum sulfide and the zinc salts of alkyl dithiophosphoric acids have been used as additives for reducing wear, such metal salts have a disadvantage in that they increase the over-all metal content of the lubricating oil. The oil composition may already be unduly high in metal content because of the presence of such detergent-inhibitors as overbased metal sulfonates, metal salts of alkyl phenol sulfides, metal carbonate dispersions, and the like. It is sometimes considered undesirable to have large quantities of metal present in a crankcase lubricant because the metal may contribute to combustion chamber deposits which promote preignition. It is self-evident that an antiwear agent which does not add to the metal content of the lubricant will have a considerable advantage. Also, there are obvious advantages for an ashless antiwear additive in a formulation where the detergent-inhibitor is of the ashless variety.

It has now been found that the mono salts (i.e. the half salts) formulated by the partial neutralization of chlorendic acid with long chain aliphatic amines of from about 12 to 24 carbon atoms are useful as ashless antiwear additives for lubricating oils. Particularly useful are the mono salt prepared from a C<sub>18</sub>—C<sub>22</sub> aliphatic amine mixture of about 300 molecular weight marketed commercially as Primene JMT by Rohm and Haas Co., and the mono salt prepared from mixed hexadecyl and octadecylamines of about 260 molecular weight marketed

## 2

by Armeen H.T. Other commercially available amines of this type include Duomeen T (sometimes identified as N-tallow-1,3-diaminopropane), Armeen CD (technical dodecylamine) and Primene 81R, which is a mixture of C<sub>15</sub> to C<sub>18</sub> aliphatic amines.

Chlorendic acid may be referred to as a dicarboxylic acid derivative of a polychlorinated cyclopentadiene. This acid may also be identified as 1,4,5,6,7,7-hexachlorobicyclo(2.2.1)-5-heptene-2,3-dicarboxylic acid and has the

10 formula

15



Chlorendic acid may be prepared by the Diels-Alder addition of maleic anhydride to hexachlorocyclopentadiene and subsequent hydrolysis.

The invention will be more readily understood when reference is made to the following examples.

## EXAMPLE 1

25 The half salt (i.e. the mono salt) of Primene JMT and chlorendic acid was prepared as follows. A solution of 0.02 mole (7.77 grams) of chlorendic acid was prepared in 100 ml. of ether and to this was added 0.02 mole (6.3 grams) of Primene JMT. The reaction was begun at room temperature but there was some temperature increase due to the exothermic nature of the reaction. The solvent was then stripped from the mixture and the mono salt was recovered as a viscous material.

## EXAMPLE 2

30 The double salt of Primene JMT and chlorendic acid was prepared in the manner of Example 1, using a ratio of 2 moles of amine to 1 mole of acid.

## EXAMPLE 3

35 The Armeen HT mono salt of chlorendic acid was prepared by dissolving 10.36 grams of Armeen HT (0.04 mole) in 100 ml. of toluene and then adding this solution to 15.54 grams (0.04 mole) of chlorendic acid. Toluene was then removed by heating the solution on a steam bath and blowing the product with air. The mono salt was recovered as a highly viscous residue.

## EXAMPLE 4

40 The Primene JMT salt of monochlorodifluoroacetic acid was prepared by adding 43.5 grams (0.33 mole) of monochlorodifluoroacetic acid to 105 grams (0.33 mole) of Primene JMT with stirring. The reaction was 45 exothermic but no external cooling was employed. The product was a red-brown thick oil.

## EXAMPLE 5

50 In the same manner as in Example 4, the Primene JMT salts of trichloroacetic acid, monochloroacetic acid, and heptafluorobutyric acid were prepared by reaction of equimolar proportions of the amine with the respective acids.

## EXAMPLE 6

55 Using as the base stock a refined mineral white oil having a viscosity of 78 centistokes at 100° F., a number of blends were prepared each containing 1 wt. percent of phenyl alpha naphthyl amine as a corrosion and oxidation inhibitor and 0.5 wt. percent of one of the salts described in Examples 1, 2, 4, and 5. Each of the compositions was subjected to an oxidation and corrosion stability test at 347° F., conducted in accordance with

Method 5308.4 of Federal Test Method Standard No. 791 as outlined in Military Specification MIL-L-7808D. The corrosion and oxidation results obtained with each of the compositions are presented in Table I. It will be noted that the chlorendic acid mono salt of the present invention exhibited low corrosion tendencies toward the various metals. Furthermore, the mono salt of the present invention showed much less oxidation promoting tendency than any of the other salts as demonstrated by the markedly lower increase in viscosity and the much lower total acid number of the oil at the end of the test.

Table I  
RESULTS OF OXIDATION AND CORROSION STABILITY TESTS AT 347° F. ON VARIOUS PRIMENE JMT SALTS OF HALOGENATED ACIDS

| Corrosion Results                          | None  | Chlorendic Acid Double Salt | Chlorendic Acid Mono Salt | Trichloro-acetic Acid | Chloro-acetic Acid | Chloro-difluoro-acetic Acid | Hepta-fluoro-butyric Acid |
|--------------------------------------------|-------|-----------------------------|---------------------------|-----------------------|--------------------|-----------------------------|---------------------------|
| Metal Wt. Change<br>mg./cm. <sup>2</sup> : |       |                             |                           |                       |                    |                             |                           |
| Cu.....                                    | +0.01 | -5.1                        | -0.42                     | -0.20                 | -0.77              | -1.02                       | -0.29                     |
| Mg.....                                    | 0     | +0.04                       | +0.05                     | +0.02                 | +0.16              | +0.02                       | +7.6                      |
| Fe.....                                    | 0     | 0                           | +0.01                     | +0.01                 | +0.04              | -0.01                       | +0.01                     |
| Al.....                                    | 0     | +0.02                       | +0.02                     | +0.02                 | +0.04              | 0                           | +0.03                     |
| Ag.....                                    | +0.03 | +0.06                       | +0.04                     | -0.04                 | +0.07              | +0.15                       | +0.04                     |
| Oxidation Results:                         |       |                             |                           |                       |                    |                             |                           |
| Vis. at 100° F., cs.....                   | 83.2  | 100.15                      | 92.6                      | 124.8                 | 123.9              | 127.4                       | 148.0                     |
| Total Acid Number.....                     | 0.64  | 3.85                        | 0.65                      | 4.11                  | 5.01               | 5.78                        | 3.48                      |

## EXAMPLE 7

Compositions were prepared using as the base oil a high viscosity index mineral oil composition containing a mixture of copolymeric type viscosity index improvers and meeting the viscosity specifications of an SAE 10W-30 motor oil. The base oil also contained 0.2 wt. percent of a pour point depressant and 0.06 wt. percent of a polyethylene glycol dioleate rust inhibitor. All of the compositions contained equal amounts of a detergent-inhibitor comprising a stabilized colloidal barium carbonate-phenate complex. One composition contained 1 wt. percent of sulfurized sperm oil; the second composition contained 1 wt. percent of the mono salt of Primene JMT and the chlorendic acid prepared as in Example 1; and the third contained the mono salt of Armeen HT and chlorendic acid prepared as in Example 3.

Each of these compositions was tested in the well-known Shell four-ball wear testing machine. The test is conducted as follows. The test lubricant is placed in the cup of the machine and heated to 200° F. The test cup contains three steel balls which are fixed in position by a screw cap. A fourth steel ball, which is held in a chuck, is pressed against the three lower balls with a force of 40 kilograms and is rotated at a speed of 600 r.p.m. for a period of 2 hours. At the end of the test, the amount of wear is determined by measuring the diameter of the wear scar on each of the three lower balls and averaging the results.

The compositions of the three blends tested and the wear results obtained are given in Table II. It will be seen that there was much less wear with the compositions containing the salts of the present invention as compared with the composition containing sulfurized sperm oil, which has been used in the past for reducing wear.

Table II  
FOUR-BALL WEAR TESTS

| Composition, Wt. Percent                      | Blend | Blend | Blend |
|-----------------------------------------------|-------|-------|-------|
|                                               | A     | B     | C     |
| Base Oil.....                                 | 93.24 | 93.24 | 93.24 |
| Detergent-Inhibitor <sup>1</sup> .....        | 5.65  | 5.65  | 5.65  |
| Primene JMT Mono Salt of Chlorendic Acid..... | 1.0   |       |       |
| Sulfurized Sperm Oil.....                     |       | 1.0   |       |
| Armeen HT Mono Salt of Chlorendic Acid.....   |       |       | 1.0   |
| Wear Scar Diam., mm.....                      | 0.386 | 0.749 | 0.352 |

<sup>1</sup> 51.8 wt. percent concentrate in mineral oil, 10.61 BaO content.

The lubricating oils to which the antiwear agents of the present invention may be added include not only mineral lubricating oils but various synthetic oils. The mineral lubricating oils may be of any preferred type including those delivered from the ordinary paraffinic, naphthenic, asphaltic or mixed base mineral crude oils by suitable refining methods. Synthetic hydrocarbon lubricating oils may also be employed. Other synthetic oils include dibasic acid esters such as di-2-ethyl hexyl sebacate, carbonate esters, glycol esters such as C<sub>13</sub> oxo acid diesters of tetraethylene glycol, and complex esters

as for example the complex ester formed by the reaction of 1 mole of sebacic acid with 2 moles of tetraethylene glycol and 2 moles of 2-ethyl hexanoic acid.

The additives of this invention are particularly applicable for use in lubricating oil compositions containing viscosity index improvers, e.g., polymethacrylates, polybutenes, etc., and detergent-inhibitors, e.g., metal sulfonates, metal alkyl phenol sulfides, metal carbonate soaps, phosphosulfurized hydrocarbon derivatives, and the like. The lubricant compositions may also contain antioxidants, e.g., phenyl-alpha-naphthylamine, bis phenols, etc., pour point depressants, dyes, and other additives for improving the properties of the compositions.

The antiwear additives of the invention may also be employed in conjunction with any of the ashless types of detergents, for example, those of the high molecular weight polymeric type having molecular weights of up to about 50,000. One example is a copolymer of 65 to 85 weight percent of mixed C<sub>9</sub>-C<sub>12</sub> fumarates, 10 to 20 weight percent of vinyl acetate, and 5 to 15 weight percent of N-vinyl pyrrolidone. Another example is the copolymer derived by reaction of mixed tallow fumarates and C<sub>8</sub> oxo fumarates, averaging about 420 molecular weight, with vinyl acetate in a 3 to 1 acetate-fumarate ratio, and 3 weight percent of maleic anhydride, followed by subsequent removal of excess vinyl acetate. By tallow fumarates is meant the esters of fumaric acid and the alcohols derived by hydrogenation of tallow. The latter are principally C<sub>16</sub> and C<sub>18</sub> alcohols with minor amounts of C<sub>12</sub>, C<sub>14</sub> and C<sub>20</sub> alcohols. C<sub>8</sub> oxo alcohols are prepared by reaction of carbon monoxide and hydrogen on mixed C<sub>3</sub>-C<sub>4</sub> olefins followed by hydrogenation of the resulting aldehydes.

The compositions embodying the additives of this invention include not only automotive crankcase lubricants but also such other lubricants and fluids as turbine oils, various industrial oils, hydraulic fluids, transmission fluids, and the like. A particular application of the additives is as a replacement for zinc salts of dialkyl dithiophosphoric acids as antiwear agents in fluids for automatic transmissions, where the zinc salts suffer the disadvantage of poor heat stability at high temperatures, e.g., 300° F. or higher. The compositions of Example 7 can serve as automatic transmission fluids for example.

The antiwear additives of this invention may be employed in lubricating compositions in concentrations ranging from about 0.01 to about 5 percent by weight, preferably about 0.1 to about 2 percent by weight.

It is to be understood that the examples presented herein are intended to be merely illustrative of the invention and not as limiting it in any manner; nor is the invention to be limited by any theory regarding its operability. The scope of the invention is to be determined by the appended claims.

What is claimed is:

1. An improved lubricating composition having superior antiwear properties which comprises a major proportion of an oil of lubricating viscosity grade into which has been incorporated from about 0.01 to about 5 weight percent of the mono salt of chlorendic acid and an aliphatic amine having in the range of from 12 to 24 carbon atoms.
2. The lubricating composition as defined by claim 1 wherein said lubricating oil is a mineral oil.
3. The lubricating composition as defined by claim 1 which includes a detergent additive.

4. The lubricating composition as defined by claim 1 wherein said amine comprises C<sub>18</sub>-C<sub>22</sub> mixed aliphatic amines of about 300 molecular weight.

5. The lubricating composition as defined by claim 1 wherein said amine comprises mixed hexadecyl and octadecyl amines.

References Cited in the file of this patent

UNITED STATES PATENTS

|    |           |              |       |               |
|----|-----------|--------------|-------|---------------|
| 10 | 2,733,248 | Lidov        | ----- | Jan. 31, 1956 |
|    | 2,771,423 | Dorinson     | ----- | Nov. 20, 1956 |
|    | 2,971,913 | David et al. | ----- | Feb. 14, 1961 |

OTHER REFERENCES

"HET Acid," Hooker Electrochemical Co., Niagara Falls, 1952, page 4.